

Apr. 10, 1923.

1,451,333

F. A. EUSTIS ET AL

ART OF MAKING ELECTROLYTIC IRON

Original Filed Dec. 1, 1920



*Inventors*

Frederic A. Eustis  
Carle R. Hayward  
Henry M. Schleicher  
Donald Belcher  
By Frank D. Dibbles & Fishman  
their Attorneys

## UNITED STATES PATENT OFFICE.

FREDERIC A. EUSTIS, OF MILTON, CARLE R. HAYWARD, OF QUINCY, AND HENRY M. SCHLEICHER AND DONALD BELCHER, OF BOSTON, MASSACHUSETTS, ASSIGNEES, BY DIRECT AND MESNE ASSIGNMENTS, OF ONE-HALF TO SAID EUSTIS AND ONE-HALF TO CHARLES PAGE PERIN, OF NEW YORK, N. Y.

## ART OF MAKING ELECTROLYTIC IRON.

Original application filed December 1, 1920, Serial No. 427,541. Divided and this application filed July 7, 1921. Serial No. 482,928.

To all whom it may concern:

Be it known that we, FREDERIC A. EUSTIS, of Milton, in the county of Norfolk, CARLE R. HAYWARD, of Quincy, in said county of Norfolk, and HENRY M. SCHLEICHER and DONALD BELCHER, both of Boston, in the county of Suffolk, all in the Commonwealth of Massachusetts, citizens of the United States of America, have invented new and useful Improvements in the Art of Making Electrolytic Iron, of which the following is a specification.

This invention relates to the manufacture of electrolytic iron from solutions, and the preparation of the ferrous solutions suitable for the electrolytic deposit of iron.

The present application is a division of an application filed by us December 1, 1920, Serial No. 427,541, now Letters Patent of the United States No. 1,412,174, dated April 11, 1922, and is addressed particularly to that modification of the invention described in our said former application employing an electric current for reducing the ferric solution in the liquor discharged from the anode compartment of the electrolytic cell in which the iron is deposited.

The ferrous solution from which iron is deposited by electrolysis may be a solution of ferrous chloride in water, a ferrous sulphate solution, or indeed a solution containing any salts of iron that will in solution dissociate to deposit iron under the action of electrolysis, that will form the two series of salts, ferric and ferrous, and that will attack the ore or other raw material constituting the source of iron. By way of illustration therefore, and not of limitation, we will describe the processes using a ferrous chloride solution.

The ferrous solution when made by the method hereinafter described will contain at least some acid or ferric salts, such as ferric chloride, although it may be only traces, and must be thoroughly neutralized before it is suitable for the production of electrolytic iron, because the presence of acid or ferric salts causes a poor iron deposit and results in low current efficiency. To this end the solution is mixed with pulverized limestone

in a suitable tank. Limestone furnishes calcium carbonate ( $\text{CaCO}_3$ ) which is the most suitable agent for neutralization, as it has the capacity of readily precipitating first ferric salts before precipitating the ferrous salts. We have found that for the best results it is advisable to use enough neutralizing agent to precipitate a small amount of ferrous iron. This insures complete neutralization of the liquor, the neutrality of the solution in the cathode compartment of the electrolytic cell being an indispensable condition for the most efficient electrolysis of iron.

The solution is then filtered if necessary heated nearly to the boiling point, and passed hot into the cathode compartment of a diaphragm electrolytic cell. Under proper conditions metallic iron is deposited on the cathode. The liquor passes through the diaphragm into the anode compartment and is thence returned to the process to be used in making more ferrous solution as hereinafter described.

The accompanying drawing illustrates diagrammatically apparatus for performing the process.

A special electrolysis cell A is used for depositing the iron, of the kind fully described in our said former patent to which reference is made for a more detailed description of its construction and mode of operation.

The hot anode liquor containing ferric chloride and ferrous chloride (or ferric and ferrous sulphates if the original solution was a sulphate instead of a chloride) is discharged from the main electrolysis cell A in which the iron is deposited, into a second electrolytic cell G which may be termed an electrolytic reducing tank. The application of electric energy to the ferric solution in the electrolytic reducing tank G, will reduce the solution from the ferric to ferrous state. This reduction of the ferric salts formed in electrolysis cell A furnishes acid needed for dissolving the ore. The ferrous solution resulting from this electrolytic reducing step constitutes a leach liquor by which the iron may be dissolved from the ore. The reduced leach liquor is then put on the ore in a solu-

tion tank B where it dissolves iron from the ore and is then filtered at C. Thence the major part of the solution is pumped back to the reducing tank G, while the smaller part of the solution which may still be slightly acid will be advanced to the limestone tank D in which it will be neutralized. The solution from the limestone tank D is then delivered hot, preferably at a temperature in the region of the boiling point, to the electrolysis cell A for the deposit of iron, and the cycle repeated.

The part of the solution sent to the limestone tank D may optionally be passed through a tank F containing scrap iron for the purpose of further enriching the solution in iron and at the same time using up part of the acid coming from the solution tank B before it enters the limestone neutralizing tank D.

It is desirable to provide agitation of some sort in the solution tank B.

The reason for returning the greater part of the liquor from the ore solution tank to the reducing cell is that the effect of the action of the leach liquor on most oxidized ores is to take iron into solution in ferric state; therefore, the solution coming from the ore solution tank will contain ferric salts and must again be reduced.

If all the liquor were sent direct to the limestone neutralizing tank it would be necessary to use large amounts of limestone for neutralization because of the large amount of ferric chloride present in the solution dissolved from the ore. This is not only costly in limestone but may use up too much acid in the neutralization step. Therefore, a part of the solution is sent from the ore solution tank back to the reducing cell where the ferric chloride dissolved from the ore is reduced, and the solution so reduced upon again passing over the ore picks up more ferric iron but only one third as much as was present immediately before it was reduced. Thus by repeatedly cycling part of the solution through the reducing tower and over the ore the ferric iron in that part of the solution advanced to the limestone tank may be diminished to any point desired.

Since no acid is added for reduction by the present method, but only electrical energy, there is no source of new acid in the cyclic process itself and the acid must therefore be carefully conserved. This can be done by turning a large portion of the solution from the ore solution tank back to the reducing cell and advancing only a small portion to the limestone tank for neutralizing. Even with this mode there is some loss of acid which can economically be restored by blowing  $\text{SO}_2$  gas into the liquor in the reducing cell or at some other convenient point.

When the reduction of the anode liquor is performed by an electrolytic reducing cell,

oxygen comes off at the anode of the reducing cell during the electrolysis if a sulphate electrolyte is used, and may be recovered as a by-product. When a chloride electrolyte is used chlorine gas is given off, and for this reason the electrolytic method of reduction is less desirable for chloride solutions than for sulphate solutions.

The ore to be treated in the solution tank B should be finely ground or pulverized to insure an efficient and speedy action of the solvent. Many oxide ores occur in nature in fine condition and such will require only a final pulverizing treatment. The mixture in the solution tank should be maintained at a high temperature, as the hotter the mixture the more effective is the action. Good results may be obtained at a temperature of 70° C. and above. It is also desirable to stir or agitate the mixture in order to insure constant contact of active solvent with the ore; or percolation may be used. A counter-current method of leaching is advised, by which fresh ore is treated with the weakest solution and the residue of the ore is treated with fresh solution.

The process above described is particularly adapted to the treatment of oxidized ores of iron, such as limonite, hematite or magnetite, as the source of iron, since the anode liquor resulting from the use of oxidized ores contains both ferric and ferrous chloride or sulphate and should be reduced to a ferrous state in order to make an effective solvent for the ore. It might also be used for the treatment of sulphide ore if the sulphide ore is of such character that the reduction of the solution will not readily take place in the solution tank along with the solution of the iron, but can better be performed as a separate step after the liquor is discharged from the electrolysis cell A and before it is put into the solution tank B.

For a further division of the aforesaid application Serial No. 427,541, reference is made to an application Serial No. 482,929, filed by us July 7, 1921.

We claim:

1. The art of making electrolytic iron which comprises reducing a ferric solution by means of an electric current to a ferrous state, and then transferring the ferrous solution to a separate electrolytic cell to which the ferric solution has no access and depositing iron from the ferrous solution by electrolysis in said separate cell.

2. The art of making electrolytic iron which comprises reducing a ferric solution by means of an electric current, leaching an iron ore with the reduced solution, and depositing iron from the leach liquor by electrolysis.

3. The art of making electrolytic iron which comprises reducing a ferric solution

by means of an electric current, leaching an oxidized iron ore with the reduced solution and depositing iron from the leach liquor by electrolysis.

4. The art of making electrolytic iron which comprises reducing a ferric solution by means of an electric current, leaching an iron ore with the reduced solution, neutralizing the solution and depositing iron therefrom by electrolysis.

5. The art of making electrolytic iron which comprises reducing a ferric solution

by means of an electric current, leaching an iron ore with the reduced solution, maintaining the solution at a temperature in the region of the boiling point and depositing iron from the solution while hot by electrolysis.

Signed by us this 5th day of July, 1921.

FREDERIC A. EUSTIS.

CARLE R. HAYWARD.

HENRY M. SCHLEICHER.

DONALD BELCHER.